

# UNITED STATES PATENT OFFICE.

NELSON PARMETER, OF GARDNER, MASSACHUSETTS.

## IMPROVEMENT IN MANUFACTURE OF BRICKS.

Specification forming part of Letters Patent No. **24,050**, dated May 17, 1859.

*To all whom it may concern:*

Be it known that I, NELSON PARMETER, of Gardner, county of Worcester, and Commonwealth of Massachusetts, have invented an Improved Fire-Proof Brick or Lining for Furnaces, Stoves, Buildings, and other Purposes; and I do hereby declare that the following is a full and exact description of the mode of making the same, so as to enable others skilled in the art to make and use it.

Sandstone, (found in the vicinity of Potsdam, St. Lawrence county, New York,) pipe-clay, and plaster-of-paris are each pulverized and sifted. Lime is slaked and also pulverized and sifted. These four materials, together with some salt, are then placed in a kettle over a fire, and water is added to it. The mixture is to be constantly stirred and kept sufficiently warm, so as to be preserved in a state of consistency similar to common mortar for striking brick. This degree of consistency is to be kept up by adding water from time to time. As much of the mixture as is wanted for immediate use is placed in a vat, and some of the coagulated blood is added to it to make it ready for use. The material is then placed into molds of such form as will suit the purpose the bricks are intended for, and the bricks are to be struck before the material cools. The bricks must then be placed under cover and dried. Pains should be taken to turn them often, so as to prevent their warping and cracking, preserve their symmetrical form, and dry them equally. The bricks, when nearly

dried, are placed in the kiln and burned, commencing with a gradual fire, and care being taken not to heat them too quick, and keeping the fire as equal as possible.

Bricks intended for nice work—such as lining hot-air furnaces, stoves, and the like—ought to be placed away from the ashes and near the middle of the stack, so as not to be exposed to the greatest heat, nor should they be placed at the top of the stack, too far from the fire.

The blood used in the above operation is put up with some salt, so as to keep in the proper state of preservation until using it.

The above-named component parts of my improved fire-proof brick or lining are used in the following proportions, according to weight: sandstone, one part; pipe-clay, one part; plaster-of-paris, one part; lime, four-eighths part; salt, two-eighths part; coagulated part of the blood, (called "crassamentum,") one-eighth part.

Having described my improved fire-proof brick or lining, what I claim therein as new, and desire to secure by Letters Patent, is—

A fire-proof brick or lining composed of the above-named ingredients, in the proportions set forth, and in the manner substantially as described.

NELSON PARMETER.

Witnesses:

THOS. H. DODGE,  
M. C. GRITZNER.